# EUROPEAN PATENT SPECIFICATION

(11) **EP 2 873 919 B1**
(45) Date of publication and mention of the grant of the patent: **09.01.2019**
(21) Application number: 14191847.4
(22) Date of filing: 05.11.2014
(51) Int. Cl.: F23Q 7/00

(54) **Glow plug**
Glühkerze
Bougie d'incandescence

(30) Priority: 15.11.2013 JP 2013237005
(43) Date of publication of application: 20.05.2015
(73) Proprietor: NGK Spark Plug Co., Ltd., Nagoya-shi, Aichi 467-8525 (JP)
(72) Inventor: Okada, Hirofumi, Nagoya-shi, Aichi 467-8525 (JP)
(74) Representative: Behr, Wolfgang

(56) References cited:
- EP-A2- 2 410 243
- JP-A- 2011 038 720

## Description

### BACKGROUND

### 1. Technical Field

The present invention relates to a glow plug.

### 2. Related Art

The glow plug includes a sheath heater. The sheath heater is employed as an auxiliary heat source for an internal combustion engine (for example, a diesel engine) by compression ignition system. Good heating characteristics or similar characteristics are required for the glow plug. To achieve this, various methods have been proposed. For example, there is known a method that controls melting of a sheath tube and a heating unit to stabilize heating characteristics of the heating unit (for example, Japanese Patent No. 4288850).

JP 2011 038720 A shows a glow plug having a sheath heater arranged in the glow plug, the sheath heater comprising a tube portion made of a nickel alloy comprising 1.0 to 2.5 mass% aluminum, and a heating coil welded to the front end portion of the tube portion, the heating coil comprising 2.0 to 4.0 mass% of aluminum.

EP 2 410 243 A2 shows a glow plug having a sheath heater arranged in the glow plug, the sheath heater comprising a sheath tube made of a nickel alloy comprising 1.0 to 2.4 mass% aluminum, and a heating coil welded to the front end portion of the tube portion, the heating coil being made from an iron - chromium - aluminum alloy.

The problem of the above-described prior art is that there is a room for improvement in durability. Usually, the sheath tube and the heating unit are formed of different materials from one another. Accordingly, at a welded portion, which is formed by welding the sheath tube and the heating unit, a new compound, which is not contained in the sheath tube or the heating unit, may be generated. If this compound has low toughness, this may cause degrade of durability of the welded portion.

### SUMMARY

The above-described problem is solved by a glow plug according to claim 1. Preferred embodiments of the present invention are the subject matter of the dependent claims.

With this glow plug, the tube portion may contain chrome at a content ratio of 24 to 26 mass%. The tube portion may contain aluminum at a content ratio of 1.8 to 2.4 mass%. According to this configuration, the above-described effect can be obtained when the content ratio of chrome of the tube portion is 24 to 26 mass% and the content ratio of aluminum of the tube portion is 1.8 to 2.4 mass%.

With this glow plug, a main constituent of the heating unit may be nickel. According to this configuration, the above-described effect can be obtained when the main constituent of the heating unit is nickel.

With this glow plug, the welded portion may contain aluminum at a content ratio of 1 mass% or less at the part near the boundary. According to this configuration, the durability of the welded portion can further be improved.

The embodiments of the present invention can be achieved in various configurations other than the above-described configurations within the scope of the appended claims.

### BRIEF DESCRIPTION OF DRAWINGS

FIG. 1 is an external view and a sectional view of a glow plug;
FIG. 2 is a sectional view of a sheath heater;
FIG. 3 is a sectional view of near front ends of a sheath tube and a heat generating coil before welding the sheath tube and the heat generating coil;
FIG. 4 illustrates a part to be analyzed near a boundary of a welded portion and a tube portion;
FIG. 5 shows a relationship between a content ratio of aluminum and generation of a crack near the boundary;
FIG. 6 is a sectional view of near front ends of a sheath tube and a heat generating coil before welding the sheath tube and the heat generating coil of another embodiment; and
FIG. 7 is a sectional view of near front ends of a sheath tube and a heat generating coil before welding the sheath tube and the heat generating coil of another embodiment.

### DETAILED DESCRIPTION

In the following detailed description, for purpose of explanation, numerous specific details are set forth in order to provide a thorough understanding of the disclosed embodiments. It will be apparent, however, that one or more embodiments may be practiced without these specific details. In other instances, well-known structures and devices are schematically shown in order to simplify the drawing.

FIG. 1 illustrates a glow plug 10. FIG. 1 illustrates an external constitution of the glow plug 10 on the right side of an axial line O on the paper. A cross-sectional structure of the glow plug 10 is illustrated on the left side of the axial line O on the paper. The glow plug 10 functions as a heat source assisting an ignition at a start of a diesel engine.

The glow plug 10 includes a center rod member 200, a metal shell 500, and a sheath heater 800. The sheath heater 800 generates heat by transmission of electricity. These members are assembled along the axial line O of the glow plug 10. In this description, the sheath heater 800 side in the glow plug 10 is referred to as a "front end side" while the opposite side is referred to as a "rear end side."

The metal shell 500 is formed into a tubular shape and made of carbon steel 1. The metal shell 500 holds the sheath heater 800 at an end portion on the front end side. The metal shell 500 holds the center rod member 200 at the end portion on the rear end side via an insulating member 410 and an O-ring 460. A position of the insulating member 410 in the axial line O direction is secured by crimping a ring 300 in contact with a rear end of the insulating member 410 to the center rod member 200. The insulating member 410 insulates the rear end side of the metal shell 500. The metal shell 500 incorporates a part of the center rod member 200 from the insulating member 410 to the sheath heater 800. The metal shell 500 includes an axial hole 510, a tool engagement portion 520, and an external thread portion 540.

The axial hole 510 is a through hole formed along the axial line O. The axial hole 510 has a diameter larger than the center rod member 200. In a state where the center rod member 200 is arranged in the axial hole 510, a space is formed between the axial hole 510 and the center rod member 200 so as to provide an electrical insulation therebetween. The sheath heater 800 is press-fitted to the front end side of the axial hole 510 and is bonded. The external thread portion 540 fits an internal thread formed at an internal combustion engine (not illustrated). The tool engagement portion 520 engages a tool (not illustrated) used for installation and removal of the glow plug 10.

The center rod member 200 includes a cylindrically-formed conductive material. The center rod member 200 is assembled along the axial line O while being inserted into the axial hole 510 of the metal shell 500. The center rod member 200 includes a center rod member front end portion 210 formed at the front end side and a connecting portion 290 formed at the rear end side. The center rod member front end portion 210 is inserted to the inside of the sheath heater 800. The connecting portion 290 is an external thread projected from the metal shell 500. The engaging member 100 is fitted to the connecting portion 290.

FIG. 2 is a sectional view illustrating a detailed constitution of the sheath heater 800. The sheath heater 800 includes a sheath tube 810, a heat generating coil 820 as a heating unit, a control coil 830, and insulating powder 840.

The sheath tube 810 extends in the axial line O direction. The sheath tube 810 is a tubular member and has a closed-front end. The sheath tube 810 incorporates the heat generating coil 820, the control coil 830, and the insulating powder 840. The sheath tube 810 includes a sheath tube front end portion 811 and a sheath tube rear end portion 819. The sheath tube front end portion 811 is an end portion formed to a rounded shape to the outside at the front end side of the sheath tube 810. The sheath tube rear end portion 819 is an end portion open at the rear end side of the sheath tube 810. The center rod member front end portion 210 of the center rod member 200 is arranged at the inside from the sheath tube rear end portion 819 to the sheath tube 810. A packing 600 and the insulating powder 840 electrically insulate the sheath tube 810 is from the center rod member 200. The packing 600 is an insulating member sandwiched between the center rod member 200 and the sheath tube 810. The sheath tube 810 is electrically connected to the metal shell 500.

The control coil 830 is a coil made of a conductive material. The control coil 830 has a temperature coefficient of electrical resistivity larger than a material forming the heat generating coil 820. As this conductive material, nickel is preferable. In addition to this, for example, the conductive material may be an alloy mainly containing cobalt or nickel. The control coil 830 is disposed inside of the sheath tube 810. The control coil 830 controls electric power supplied to the heat generating coil 820. The control coil 830 includes a control coil front end portion 831 and a control coil rear end portion 839. The control coil front end portion 831 is at the end portion on the front end side. The control coil rear end portion 839 is at the end portion on the rear end side. The control coil front end portion 831 is electrically connected to the heat generating coil 820 by being welded to a heat generating coil rear end portion 829 of the heat generating coil 820. The control coil rear end portion 839 is electrically connected to the center rod member 200 by being bonded to the center rod member front end portion 210 of the center rod member 200.

The insulating powder 840 is powder having an electrical insulating property. As the insulating powder 840, for example, powder of Magnesium Oxide (MgO) is employed. The insulating powder 840 is filled inside of the sheath tube 810. The insulating powder 840 electrically insulates respective clearances of the sheath tube 810, the heat generating coil 820, the control coil 830, and the center rod member 200.

The heat generating coil 820 is a coil made of a conductive material. The heat generating coil 820 is disposed at the inside of the sheath tube 810 along the axial line O direction. The heat generating coil 820 is generates heat by transmission of electricity. The heat generating coil 820 includes a heat generating coil front end portion 821 and the heat generating coil rear end portion 829. The heat generating coil front end portion 821 is at the end portion on the front end side. The heat generating coil rear end portion 829 is at the end portion on the rear end side. The heat generating coil front end portion 821 is electrically connected to the sheath tube 810 by being welded to a part near the front end of the sheath tube 810.

FIG. 3 is a sectional view of near front ends of the sheath tube 810 and the heat generating coil 820 before welding the sheath tube 810 and the heat generating coil 820. The front end of the sheath tube 810 is open before being welded with the heat generating coil 820. The heat generating coil 820 is arranged so as to penetrate an opening end of the sheath tube 810 before welding. The front end of the heat generating coil 820 before the welding extends obliquely with respect to the axial line O as illustrated in FIG. 3. Welding the sheath tube 810 and the heat generating coil 820 at the arrangements forms the part near the front end to the shape as illustrated in FIG. 2. In this embodiment, this welding is achieved by arc welding.

FIG. 4 is a sectional view of near a welded portion 850 after welding the sheath tube 810 and the heat generating coil 820. The welded portion 850 is formed such that the heat generating coil 820 and the sheath tube 810 are mixed in a melted state, and the thus-melted portion hardens. The welded portion 850 is hatched in FIG. 4. The outer surface of the welded portion 850 forms the sheath tube front end portion 811. A tube portion 860 illustrated in FIG. 4 is a remaining part excluding the welded portion 850 from the sheath tube 810. Thus, the welded portion 850 is formed by welding. In view of this, the welded portion 850 at least contains the main constituent of the heat generating coil 820 and the main constituent of the tube portion 860.

Using FIG. 4, the following describes a constituent analysis of the welded portion 850. This analysis is performed as a preparation of experiment described later. The part to be analyzed is near the boundary between the welded portion 850 and the tube portion 860.

The part to be analyzed is determined as follows. At the left side with respect to the axial line O in FIG. 4, a point A and a point B are determined. The point A is at a most front end side on the interface of the welded portion 850 and the tube portion 860. The point B is a most rear end side on the interface. Afterwards, a straight line W passing through the point A and the point B is drawn. This straight line W is not limited to the interface between the welded portion 850 and the tube portion 860. Assuming that the axial line O is the Y-axis on the XY plane, the front end side is a positive direction of the Y-axis, and the rear end side is a negative direction of the Y-axis, the left side of the axial line O corresponds to the negative direction of the X-axis.

The interface between the welded portion 850 and the tube portion 860 is, for example, determined as follows. First, a cross section near the welded portion 850 is mirror-finished. Then, electrolytic etching is performed with oxalic acid dehydrate on this cross section. Then, based on an enlarged image of this cross section, the interface between the welded portion 850 and the tube portion 860 is visually determined.

A straight line X obtained by translating a straight line W to the axial line O side by 0.3 mm is drawn. A part of the welded portion 850 along the straight line X is linearly (along the straight line X) analyzed at 10 µm-intervals. An average value of content ratios of aluminum at the respective points, which are obtained by this analysis, is calculated as a content ratio of aluminum near the boundary. However, at a part up to 0.03 mm from the surface of the welded portion 850 is more likely to contain an oxide film. In view of this, this part is excluded from the analysis result.

Similarly, at the right side with respect to the axial line O in FIG. 4, a point C and a point D are determined. The point C is at a most front end side on the interface of the welded portion 850 and the tube portion 860. The point D is a most rear end side on the interface. Afterwards, a straight line Y passing through the point C and the point D is drawn. Furthermore, a straight line Z obtained by translating the straight line Y to the axial line O side by 0.3 mm is drawn. A part of the welded portion 850 along the straight line Z is linearly (along the straight line Z) analyzed at 10 µm-intervals. However, at a part up to 0.03 mm from the surface of the welded portion 850 is more likely to contain an oxide film. In view of this, this part is excluded from the analysis result.

The reason for determining the analysis part as described above is that these parts are likely to generate a crack. Here, the crack means a rift generated at the interface. An intermetallic compound having low toughness is likely to occur near the boundary between the welded portion 850 and the tube portion 860. Moreover, the intermetallic compound has thermal expansion characteristics different from the original metal. In addition to this, the part near the boundary is mechanically fragile. In view of this, repeated thermal expansion and thermal shrinkage may generate a crack at the interface near the boundary. This embodiment employs the above-described part as one example of the part near the boundary.

The following describes a procedure of the analysis. As the first step, using WDS of EPMA, the qualitative analysis of the welded portion 850 is performed. This analysis specifies an element contained in the welded portion 850. This analysis also specifies an element having the maximum mass% as the main constituent. The EPMA refers to an Electron Probe Micro Analyzer. The WDS refers to a Wavelength Dispersive X-ray Spectrometer.

As a second step, a measuring condition for the EPMA is determined. This is determined to enhance analysis accuracy. For example, when analyzing (detecting) an element specified as the main constituent at the first step by the amount of beam current, the measuring conditions for the EPMA includes: the amount of beam current does not cause a count loss due to incident of a large amount of X-rays and the number of measured counts of 10000 counts or more is obtained.

As a third step, the element specified at the first step is quantitatively-analyzed under the conditions determined at the second step. The above-described average value regarding the plurality of analysis target points is calculated as the content ratio of aluminum. In this analysis, the accelerating voltage was set to 20 kV, a probe current was set to 2.5 × 10⁻⁸A, and an irradiation diameter of the beam was set to 10 µm. The main peak is taken in for 10 seconds. Furthermore, backgrounds on respective high angle side and low angle side are taken in for five seconds. From net strength, a Count Per Second (CPS) of each element is obtained. Using this CPS and the CPS of a comparative sample (standard sample manufactured by Astimex Standards Ltd.) analyzed under the same conditions, a quantitative calculation is performed by a ZAF method. The content ratio of aluminum in this comparative sample was preliminary analyzed. The ZAF is an acronym based on an atomic number effect (Z effect), absorption effect, and a fluorescence excitation effect. During this quantitative calculation, normalization (standardization) is performed such that the sum of the content ratio becomes 100%.

FIG. 5 is a table showing an experimental result regarding the relationship between a content ratio of aluminum and generation of a crack at the above-described part near the boundary.

For Experiment No. 1, the heat generating coil 820 formed by a material containing nickel as the main constituent and also containing chrome, but not containing aluminum was employed. In this description, the expression of "not containing aluminum" includes the case where aluminum is contained at the content ratio of around a level of an error. In the case of Experiment No. 1, the tube portion 860 formed by a material not containing aluminum (for example, SUS310S) was employed. As a result, the content ratio of aluminum of the welded portion 850 (part near the boundary of the tube portion 860 and the welded portion 850) in Experiment No. 1 was 0.00 mass%.

In the cases of Nos. 2 to 10, the heat generating coil 820 formed by a material containing iron as the main constituent and also containing chrome and aluminum was employed. Furthermore, the tube portion 860 formed by Alloy 602 was employed. Alloy 602 means a DIN2.4633 alloy specified by Deutsche Industrie Normen (DIN) at the time of this application. The Alloy 602 has the content ratio of chrome of 24 to 26 mass% and the content ratio of aluminum is 1.8 to 2.4 mass%. Consequently, the content ratio of aluminum of the welded portion 850 (part near the boundary between the welded portion 850 and the tube portion 860) became 3.00 to 5.50 mass%. The content ratio of aluminum of the welded portion 850 (part near the boundary of the welded portion 850 and the tube portion 860) was changed by adjusting the front end shape of the heat generating coil 820 before melting and the content ratio of aluminum contained in the heat generating coil 820.

As an experiment determining durability, in the case where thermal shock was repeatedly applied as a load, whether a crack occurred in the welded portion 850 or not was confirmed. As the load of the thermal shock, heating and cooling were conducted on the glow plug 10 by 8000 cycles. The heating was conducted for 20 seconds such that the surface of the glow plug 10 became 1150°C. The cooling was conducted for 60 seconds under the condition that the glow plug 10 was reduced by 149°C after one second from the start of cooling. These values as experimental conditions were all illustrative and therefore may be changed for reproductive experiment. For example, a temperature width lowered after one second from the start of cooling may be 139 to 159°C. A surface temperature of the glow plug 10 in the heating may be 1140 to 1160°C.

As illustrated in FIG. 5, Experiment Nos. 1 to 6 did not generate a crack. Experiment Nos. 7 to 10 generated a crack. Accordingly, the content ratio of aluminum in the welded portion 850 (part near the boundary between the welded portion 850 and the tube portion 860) is preferable to be less than 5.00 mass% and more preferable to be 4.95 mass% or less.

Furthermore, to minimize generation of the intermetallic compound from aluminum and another metal (for example, Ni₃Al, which is a compound of aluminum and nickel contained in Alloy 602), the smaller the content ratio of aluminum in the welded portion 850 (part near the boundary of the welded portion 850 and the tube portion 860) is, the more preferable the content ratio is. This content ratio is, for example, preferable to be 2.00 mass% or less and more preferable to be 1.00 mass% or less.

The techniques of the present invention are not limited to the above-described embodiments. The techniques of the present invention may be practiced in various forms without departing from its spirit and scope. For example, to solve a part of or all of the above-described problems, or to achieve a part of or all of the above-described effects, the technical features in the embodiments corresponding to the technical features in the respective embodiments described in SUMMARY may be, as necessary, replaced or combined. If the technical feature is not described as essential in the description, it can be deleted as necessary. As another embodiment in the present invention, for example, the following embodiments are illustrative.

FIG. 6 illustrates shapes of the sheath tube 810 and a heat generating coil 820a before welding the sheath tube 810 and the heat generating coil 820a as another embodiment. The heat generating coil 820a substitutes for the heat generating coil 820 in the embodiment. The front end of the heat generating coil 820a, as illustrated in FIG. 6, extends almost parallel to the axial line O.

FIG. 7 illustrates shapes of the sheath tube 810 and a heat generating coil 820b before welding the sheath tube 810 and the heat generating coil 820b as yet another embodiment. The heat generating coil 820b substitutes for the heat generating coil 820 in the embodiment. The front end of the heat generating coil 820b, as illustrated in FIG. 7, is formed such that the part projecting from the opening end is closely coiled. Besides, the shape of the heat generating coil before welding may have a different shape from the heat generating coils illustrated in FIG. 3, FIG. 6, and FIG. 7.

The material of the heat generating coil may have nickel as the main constituent. In the present invention, the welded portion means the tube portion extending in an axial direction and disposed at the outer circumference of the heating unit, and a part that contains at least the main constituent of the tube portion and the main constituent of the heating unit and blocks the front end of the tube portion.

The foregoing detailed description has been presented for the purposes of illustration and description. Many modifications and variations are possible in light of the above teaching. It is not intended to be exhaustive or to limit the subject matter described herein to the precise form disclosed. Although the subject matter has been described in language specific to structural features and/or methodological acts, it is to be understood that the subject matter defined in the appended claims is not necessarily limited to the specific features or acts described above. Rather, the specific features and acts described above are disclosed as example forms of implementing the claims appended hereto.

## Claims

1. A glow plug (10), comprising:
a heating unit (820) that generates heat by transmission of electricity; and
a sheath tube (810) including a tube portion (860) and a welded portion (850), the tube portion (860) being disposed at an outer circumference of the heating unit (820) and extending in an axial direction, the welded portion (850) containing at least a main constituent of the tube portion (860) and a main constituent of the heating unit (820) and closing a front end of the tube portion (860), wherein
the tube portion (860) contains aluminum at a content ratio of more than 1.7 mass% and the heating unit (820) does not contain aluminum, and
the welded portion (850) contains aluminum at a content ratio of less than 2 mass% at a part near a boundary with the tube portion (860), wherein this content ratio is calculated as an average value of content ratios of aluminum on a straight line (X) analyzed at 10 µm intervals, the straight line (X) obtained by translating a straight line (W) passing through a point (A) located at a most front end side on the interface of the welded portion (850) and the tube portion (860) and a point (B) located at a most rear end side on the interface of the welded portion (850) and the tube portion (860) to an axial line (O) side by 0.3 mm, with a part of 0.03 mm from the surface of the welded portion 850 being excluded.

2. The glow plug (10) according to claim 1, wherein
the tube portion (860) contains chrome at a content ratio of 24 to 26 mass %, and contains aluminum at a content ratio of 1.8 to 2.4 mass%.

3. The glow plug (10) according to any one of claims 1 or 2, wherein
a main constituent of the heating unit (820) is nickel.

4. The glow plug (10) according to any one of claims 1 to 3, wherein
the welded portion (850) contains aluminum at a content ratio of 1 mass% or less at the part near the boundary.

## Patentansprüche

1. Glühkerze (10), aufweisend:
eine Heizeinheit (820), die Wärme durch Übertragung von Elektrizität erzeugt; und
ein Schutzrohr (810) mit einem Rohrabschnitt (860) und einem Schweißabschnitt (850), wobei der Rohrabschnitt (860) an einem Außenumfang der Heizeinheit (820) angeordnet ist und sich in einer Axialrichtung erstreckt, wobei der Schweißabschnitt (850) zumindest einen Hauptbestandteil des Rohrabschnitts (860) und einen Hauptbestandteil der Heizeinheit (820) enthält und ein vorderes Ende des Rohrabschnitts (860) verschließt, wobei
der Rohrabschnitt (860) Aluminium mit einem Anteilsverhältnis von mehr als 1,7 Massenprozent enthält, und die Heizeinheit (820) kein Aluminium enthält, und
der Schweißabschnitt (850) Aluminium mit einem Anteilsverhältnis von weniger als 2 Massenprozent an einem Teil nahe einer Grenze zu dem Rohrabschnitt (860) enthält, wobei dieses Anteilsverhältnis als Durchschnittswert von Anteilsverhältnissen von Aluminium auf einer Geraden (X), analysiert mit Abständen von 10 µm, berechnet wird, wobei die Gerade (X) durch Verlagerung einer Geraden (W), die durch einen Punkt (A), der sich an einer vordersten Endseite an der Grenzfläche des Schweißabschnitts (850) und des Rohrabschnitts (860) befindet, und einen Punkt (B) verläuft, der sich an einer hintersten Endseite an der Grenzfläche des Schweißabschnitts (850) und des Rohrabschnitts (860) befindet, hin zu einer Seite einer axialen Linie (O) um 0,3 mm erhalten wird, wobei ein Teil von 0,03 mm von der Oberfläche des Schweißabschnitts (850) ausgenommen ist.

2. Glühkerze (10) nach Anspruch 1, wobei
der Rohrabschnitt (860) Chrom mit einem Anteilsverhältnis von 24 bis 26 Massenprozent enthält, und Aluminium mit einem Anteilsverhältnis von 1,8 bis 2,4 Massenprozent enthält.

3. Glühkerze (10) nach einem der Ansprüche 1 oder 2, wobei
ein Hauptbestandteil der Heizeinheit (820) Nickel ist.

4. Glühkerze (10) nach einem der Ansprüche 1 bis 3, wobei
der Schweißabschnitt (850) Aluminium mit einem Anteilsverhältnis von 1 Massenprozent oder weniger an dem Teil nahe der Grenze enthält.

## Revendications

1. Bougie de préchauffage (10), comprenant :
une unité de chauffage (820) qui génère de la chaleur par transmission d'électricité ; et
un tube de gaine (810) comprenant une partie de tube (860) et une partie soudée (850), la partie de tube (860) étant disposée au niveau d'une circonférence externe de l'unité de chauffage (820) et s'étendant dans une direction axiale, la partie soudée (850) contenant au moins un constituant principal de la partie de tube (860) et un constituant principal de l'unité de chauffage (820) et fermant une extrémité avant de la partie de tube (860),
la partie de tube (860) contenant de l'aluminium à un rapport en teneur supérieur à 1,7 % en masse et l'unité de chauffage (820) ne contenant pas d'aluminium, et
la partie soudée (850) contenant de l'aluminium à un rapport en teneur inférieur à 2 % en masse au niveau d'une partie proche d'une limite avec la partie de tube (860), ce rapport en teneur étant calculé comme une valeur moyenne de rapports en teneur d'aluminium sur une ligne droite (X) analysés à des intervalles de 10 µm, la ligne droite (X) étant obtenue par translation d'une ligne droite (W) passant par un point (A) situé au niveau d'un côté le plus en avant sur l'interface de la partie soudée (850) et de la partie de tube (860) et un point (B) situé au niveau d'un côté le plus en arrière sur l'interface de la partie soudée (850) et de la partie de tube (860) vers un côté ligne axiale (O) de 0,3 mm, une partie de 0,03 mm depuis la surface de la partie soudée (850) étant exclue.

2. Bougie de préchauffage (10) selon la revendication 1, dans laquelle
la partie de tube (860) contient du chrome à un rapport en teneur de 24 à 26 % en masse, et contient de l'aluminium à un rapport en teneur de 1,8 à 2,4 % en masse.

3. Bougie de préchauffage (10) selon l'une quelconque des revendications 1 ou 2, dans laquelle
un constituant principal de l'unité de chauffage (820) est le nickel.

4. Bougie de préchauffage (10) selon l'une quelconque des revendications 1 à 3, dans laquelle
la partie soudée (850) contient de l'aluminium à un rapport en teneur de 1 % en masse ou moins au niveau de la partie proche de la limite.
